

Oct. 27, 1931.

H. E. COLEY

1,829,438

REDUCTION OF ORES, OXIDES, AND THE LIKE

Filed Jan. 5, 1931

4 Sheets-Sheet 1



Fig. 1.

INVENTOR.  
H. E. COLEY.

By Blair & Kilroy, ATTYS.

Oct. 27, 1931.

H. E. COLEY

1,829,438

REDUCTION OF ORES, OXIDES, AND THE LIKE

Filed Jan. 5, 1931

4 Sheets-Sheet 2



Fig. 3.



Fig. 2.



Fig. 4.

INVENTOR  
H. E. COLEY.

By Alan Kilroyne.  
ATTYS.

Oct. 27, 1931.

H. E. COLEY

1,829,438

REDUCTION OF ORES, OXIDES, AND THE LIKE

Filed Jan. 5, 1931

4 Sheets-Sheet 3



Fig. 5.

INVENTOR.  
H.E. COLEY.

By Blair Kilcoyne.  
ATTYS.

Oct. 27, 1931.

H. E. COLEY

1,829,438

REDUCTION OF ORES, OXIDES, AND THE LIKE

Filed Jan. 5, 1931

4 Sheets-Sheet 4



*Fig. 6.*



*Fig. 7.*  
INVENTOR,  
H.E. COLEY,  
By *Blair Kilcorme*,  
ATTYS.

## UNITED STATES PATENT OFFICE

HENRY EDWIN COLEY, OF LONDON, ENGLAND

REDUCTION OF ORES, OXIDES, AND THE LIKE

Application filed January 5, 1931. Serial No. 506,731.

This invention relates to the reduction of ores, oxides and the like. The invention is particularly adapted for reducing zinc ores, although it is to be distinctly understood that it is applicable also to many other kinds of ores as well.

One of the objects of the invention is to provide a new method of internally heating the chamber in which reduction of the material is effected consisting in cracking a hydrocarbon by bringing it into contact with heated ore, oxide or the like within the reducing chamber and burning the combustible vapours produced by means of separately introduced air. A further object of the invention is to utilize a hydrocarbon to effect both the heating of the material to be reduced and its reduction contemporaneously by cracking the hydrocarbon by bringing it into contact with a body of the ore, oxide or the like heated to its reducing temperature and admitting air to the region where such cracking takes place sufficient to effect combustion of the combustible vapours produced and the production of a non-oxidizing atmosphere.

By means of this method reduction of the ore or the like is effected by means of nascent carbon or carbon in its atomic condition as distinct from carbon in its ordinary or molecular condition whilst by the separate admission of just sufficient air for the purpose in the region where the cracking of the hydrocarbon takes place the combustible vapours given off are burnt without producing an oxidizing atmosphere.

Apparatus suitable for carrying the invention into effect is illustrated in the accompanying drawings in which:—

Fig. 1 is a longitudinal vertical section through a reducing chamber of the rotatable tube type adapted for reducing volatile metals such as zinc and embodying means for introducing a hydrocarbon and air for carrying the present invention into effect.

Fig. 2 is a fragmentary section to an enlarged scale of the means illustrated in Fig. 1 for introducing a non-cracked hydrocarbon into the body of ore or the like in the reducing chamber.

Figs. 3 and 4 illustrate a means for clear-

ing the outlets of the hydrocarbon feed pipes.

Fig. 5 is a transverse vertical section to an enlarged scale through the hydrocarbon feeding mechanism illustrated in Fig. 1.

Fig. 6 is a fragmentary vertical section of the same reducing chamber illustrating a modified means for introducing the air for combustion.

Fig. 7 is a transverse section on an enlarged scale through the reducing chamber illustrated in Fig. 1 showing two positions of the air inlet pipes and the operation of the automatic valves controlling the inlet end of such pipe.

Referring to the drawings the reducing chamber illustrated is in the form of a rotatably mounted tube 1 having openings 2 and 3 at opposite ends, said openings being suitably sealed against the free ingress of air the opening 2 being for the removal of the vaporous products of reduction and the opening 3 for the removal, by way of the chute 4 of the gangue or residue. The ore, a bank of which is indicated at 5 in position along the interior of the reducing chamber is fed in by way of the opening 2 by means comprising an inclined chute 6, a communicating horizontal or substantially horizontal tube 7 and a worn or other conveyor 8. These ore feeding means are supported by and extend through a water-jacketed tower 9 in which is effected the condensation of the metallic vapours and their separation from the other gases produced by the reduction as described in the specification of my pending application for Letters Patent No. 301,889. Extending longitudinally through the centre of the reducing tube is a stationary tube or hollow girder 10 which is supported at opposite ends by supports 11 and 12. Through the interior of this tube or girder water is continuously circulated, the inlet for such water being at one end and indicated at 13 and the outlet at the opposite end, being indicated at 14, such outlet discharging into the interior of the aforesaid condensing tower 9.

Extending radially and at spaced intervals from the tube or girder 10 are a plurality of nozzles, the construction of which is indicated clearly in Fig. 2. These nozzles com-

prise a comparatively small inner tube 15 each of which is water-jacketed to its extremity by means comprising inner and outer spaced tubes 16 and 17, the latter tube closing 5 in against the extremity of the small inner tube 15. The interior of the tube 16 communicates with the interior of the tube or girder 10 by means of an inlet opening 16a and similarly the interior of the outer tube 17 also 10 communicates with the interior of the tube or girder 10 by means of an outlet passage 17a. Water from the interior of the tube or girder 10 is thus caused to circulate through the spaces formed by means of the concentric 15 tubes 16 and 17 in the direction of the arrows shown in Fig. 2. The inner small tube 15 is thus always maintained comparatively cool. As an additional precaution in this direction the outer tube 17 is enclosed by means of an 20 outside casing 18 having an interposed packing 19 of any suitable heat insulating material.

The inner tubes 15 which at their extremities open into the interior of the reducing 25 chamber are adapted to deliver, in a non-cracked and comparatively cool condition, a liquid hydrocarbon and for this purpose each such tube communicates at its inner end with a tube 20 which latter tubes extend longitudinally 30 through the water space within the interior of the tube or girder 10. These tubes 20 project through the left hand end closure of the tube or girder 10 and are thus outside of the reducing chamber and such exposed 35 extremities are each fitted with feed or inlet pipes 21 communicating with the main hydrocarbon supply.

As will be seen from Fig. 5 the water-cooled hydrocarbon supply nozzles extend 40 into the interior of the reducing chamber at an angle to the vertical so that during the rotation of the reducing tubes the outlets of these nozzles are always normally covered by the bank of ore.

45 Means are provided, in the example illustrated, for preventing the outlets of the hydrocarbon delivery pipes or tubes 15 from becoming choked with coke such means comprising pricker rods 22 which extend down 50 through the centre of each such pipe 15 and are adapted to be periodically reciprocated by means of a crank connection 23 between such pricker rods and further rods 24 located within the longitudinal feed tubes or pipes 20 55 which latter rods may be oscillated or partially rotated for the purpose from their outer extremities 25.

As shown in Fig. 5 the water-cooled tube or girder 10 may be additionally protected 60 against the radiant heat within the reducing chamber by means of an exterior shrouding 26 and an interposed packing 27 of a suitable non-conducting material.

By these means a liquid hydrocarbon is 65 conveyed in a non-cracked condition into

actual contact with a bank of ore heated to its reducing temperature. As a result of the contact between the comparatively cool hydrocarbon and the hot ore the hydrocarbon is cracked in situ producing carbon in its 70 most active form, namely, in its atomic or nascent form and in this form effects the reduction of the ore.

When a hydrocarbon is cracked there are given off a quantity of combustible gases 75 which it is one of the objects of this invention to use for the purpose of heating the ore to and maintaining it at its reducing temperature within the reducing chamber. This object is attained according to the present invention by separately introducing air into the reducing chamber in proximity to the region or regions where the cracking of the hydrocarbon takes place the quantity of air thus admitted being sufficient to effect complete 80 combustion of the said combustible gases without producing an oxidizing atmosphere within the reducing chamber. In the arrangement illustrated in Figs. 1, 2, 3, 4, 5 and 7 this air is introduced into the interior of the 85 reducing chamber by means of a plurality of tubes 28 which extend radially through the wall of the reducing chamber. In practice it is found to be essential to prevent this air from being projected directly onto the exposed surface of the bed of hot ore and to this end the outer end of each tube is provided with a flap valve 29 each of which is hinged at 30 a stop 31 being provided to limit their opening movement. These valves thus operate by gravity and remain closed until the rotation of the reducing chamber brings the tubes to a position where their inner ends project through the bank of hot ore as shown most clearly in Fig. 7. In this position of 90 the reducing chamber the valves fall open automatically and allow air to enter and by reason of the particular location of the air tubes relatively to the hydrocarbon inlets, to support combustion of the combustible 95 gases evolved by the cracking in situ of the introduced hydrocarbon. During the remaining revolution of the reducing chamber the valves 29 remain closed.

In the modified arrangement illustrated 100 in Fig. 6 the air is introduced by means of a plurality of longitudinal tubes 32 of varying lengths. As the outlets of these tubes serve to discharge the air away from the bank of hot ore the provision of controlling valves as 110 in the former arrangement, is rendered unnecessary.

What I claim is:—

1. In the reducing of ores, oxides and the like effecting the reduction by bringing a 115 hydrocarbon in a non-cracked condition into contact with material to be reduced which has been heated to its reducing temperature by keeping the same artificially cooled whereby such hydrocarbon is cracked by reason of 120

contact with such heated material and maintaining the reducing temperature of the material by burning the combustible vapours produced by the cracking of the hydrocarbon with separately introduced air.

5 2. A method of reducing ores, oxides, and the like comprising the steps, charging the retort with the material to be treated, heating the same to a cracking temperature for a hydrocarbon, introducing a liquid hydrocarbon into the retort, artificially cooling the same during its introduction into the retort whereby it reaches the heated material in a non-cracked condition and is thereby cracked

10 15 by contact with the heated material and maintaining the temperature within the retort by burning the resulting combustible vapours by separately introduced air.

3. A method of internally heating retorts 20 for the reduction of ores and the like and simultaneously reducing such ores comprising the steps charging the retort with the material to be reduced, heating the material in a reducing atmosphere to a temperature at 25 which a hydrocarbon will crack introducing a hydrocarbon into the retort, artificially cooling the same during its introduction into the retort whereby it reaches the heated material in a non-cracked condition and is thereby cracked by contact with the heated material and burning the resulting combustible vapours within the retort by separately introduced air so as to heat the material to its reducing temperature, without destroying 30 the reducing atmosphere within the retort, 35 and cause reduction to be effected.

4. In the reducing of ores, and the like effecting the reduction by bringing a liquid hydrocarbon in a non-cracked condition into 40 contact with the material to be reduced, which has been heated to its reducing temperature in a reducing atmosphere, by means of a water-cooled conveyor whereby said hydrocarbon is cracked by its contact with the 45 heated material and maintaining the reducing temperature of the material by burning the combustible vapours, produced by the cracking, with separately introduced air.

Signed at London, England, this 18th day 50 of December, 1930.

HENRY EDWIN COLEY.